

## UNITED STATES PATENT OFFICE

2,304,881

## TREATMENT OF CAST IRON

Charles O. Burgess, Niagara Falls, N. Y., and Herman C. Aufderhaar, Chicago, Ill., assignors to Electro Metallurgical Company, a corporation of West Virginia

No Drawing. Application September 30, 1941,  
Serial No. 413,008

3 Claims. (CL 75—139)

The invention relates to the manufacture of cast iron and provides a new and useful method of treatment whereby the properties of the iron are improved.

A disadvantage of cast iron which has limited its use in the past is its "wall-sensitivity," that is, sensitivity to variations in wall thickness or rate of cooling. An effect of this wall-sensitivity is that an iron which is desirably soft in heavy sections is undesirably hard, or "chilled," in light sections. Considerable attention has accordingly been directed toward decreasing the sensitivity of cast iron to variations in cooling rate. Of the expedients proposed to attain this end, many involve the addition to a molten bath of cast iron of agents called "graphitizers," which usually contain elements which not only promote the formation of graphitic carbon in the iron but also combine avidly with oxygen.

The improvement obtained by the addition to molten cast iron of a graphitizer in an amount sufficient substantially to eliminate sensitivity to changes in cooling rate in the iron is sometimes accompanied by the production of minute, sometimes microscopic, subcutaneous voids or "pinholes" in the iron. Such voids are quite different from imperfections arising from improper casting procedure; an iron containing them is said to have "pinhole porosity." Pinhole porosity is particularly troublesome because it is not usually evident from surface inspection of a casting.

In general, cast iron is broadly divided into two classes, hard iron and soft iron. Whether an iron of a given carbon content is hard or soft depends in large measure upon its silicon content. Thus, an iron containing about 3% carbon and 1% silicon is hard, whereas an iron containing about 3% carbon and 3% silicon is soft. A polished and etched specimen of a hard iron has a mottled appearance; a similar specimen of a soft iron has a gray appearance. Hard irons are particularly sensitive to variations in cooling rate and are materially benefited by the addition of a graphitizer before casting. Soft irons, while not so sensitive to variations in cooling rate, are also benefited by the addition of a graphitizer. Both types of iron may develop pinhole porosity when cast after a graphitizing agent has been added; soft irons are particularly susceptible to pinhole formation.

A principal object of the invention is a method of decreasing the sensitivity of cast iron to variations in cooling rate without developing pinhole porosity in the iron. A more specific object is a method of treating molten cast iron to prevent

the formation of pinhole porosity in the iron when it is cast.

These objects are achieved by the invention which is a method of treating molten cast iron comprising temporarily raising the oxygen content of the molten iron in conjunction with, and preferably just prior to or simultaneously with, the addition of a graphitizer containing a small amount of aluminum and one or more strongly deoxidizing graphitic-carbon promoting elements. Suitably the oxygen content of the cast iron is raised by the addition to it of a readily reducible metallic oxide, preferably in the ladle or cupola forehearth just before the iron is cast, and conveniently in admixture with the graphitizing agent. Oxides which may be used include iron oxide, nickel oxide, manganese oxide, and chromium oxide, preferably in finely divided form. If iron oxide is used, convenient sources are iron ore and mill scale.

Practically all of the graphitizers in common use for the treatment of cast iron contain aluminum either as an impurity or as an intentionally added element. It was at first believed that aluminum alone was responsible for the development of pinhole porosity in cast iron, but it has been observed that the tendency of an iron to develop pinhole porosity is most pronounced when a graphitizer containing aluminum with other highly effective deoxidizing elements is used. When graphitizers containing less effective deoxidizing elements are used, the tendency toward pinhole formation in the treated iron is less. However, graphitizers of the latter type have less chill-reducing power than graphitizers containing more effective deoxidizers.

Typical graphitizers which are used for the treatment of molten cast iron include ferrosilicons, modified ferrosilicons containing about 0.25% to 10% aluminum with or without about 0.5% to 10% of one or more of the metals calcium, zirconium, and manganese, ferrosilicons containing about 1% to 16% calcium and 1% to 25% vanadium or titanium or both, and calcium-silicon alloys. As before stated, practically all of these graphitizers contain some aluminum; it is usually present in a proportion at least about 0.25%. Graphitizers are usually added to molten iron in an amount sufficient to add about 0.1% to 1.5% silicon to the iron.

In accordance with the invention there is added to molten cast iron in conjunction with the addition of a graphitizer, such as an alloy of the above-mentioned group, oxygen in an

amount between about  $\frac{1}{2}$  and 5 times the amount theoretically necessary to combine with all of the aluminum in the graphitizer to form aluminum oxide ( $Al_2O_3$ ). Because the tendency of an iron to develop pinhole porosity depends on the composition of the iron, the amount and composition of the graphitizer used, and melting conditions, the amount of oxygen to be added in a specific instance must be determined empirically. Generally, the softer the iron being treated or the more effective as a deoxidizer the graphitizer used, the more oxygen should be added. Ordinarily, when a soft iron is to be treated with a complex graphitizer containing strong deoxidizing elements, the addition of about  $\frac{1}{2}$  to 2 times the amount of oxygen theoretically required to combine with all of the aluminum in the graphitizer will be sufficient to inhibit the formation of pinhole porosity without detrimentally affecting the chill-reducing power of the graphitizer.

Tests of the method of the invention have demonstrated its effectiveness in substantially eliminating the formation of pinhole porosity in cast irons even when such irons have been treated while molten with excessive amounts of graphitizers containing strongly deoxidizing elements. In such tests several cast irons were made. Some were given a graphitizing treatment, some were given the treatment of the invention, and others were given no treatment. Standard test specimens were cast from the irons and were tested for strength, hardness, depth of chill and evidence of pinhole porosity. In the following examples typical results obtained in such tests are set forth:

**Example 1.**—Three heats of a soft iron containing about 3.5% carbon, 3% silicon and 0.6% manganese were made in a high-frequency furnace. One heat was cast without ladle additions, the ingredients simply being melted together. This iron as cast had an ultimate tensile strength of 19,500 pounds per square inch and a Brinell hardness number of 134. The depth of chill measured on a standard chill block was 0.13 inch, and there was no evidence of pinhole porosity.

A second heat was made in which 0.75% silicon was added just before casting by a ladle addition of an iron-silicon-zirconium-manganese alloy containing 2.6% aluminum. This iron as cast had an ultimate tensile strength of 24,300 pounds per square inch, and its Brinell hardness number was 146. The depth of chill was 0.06 inch and considerable pinhole porosity was evident.

A third heat was made in which 0.75% silicon was added in the ladle by the use of the same deoxidizer used in the second heat but mixed with a finely-ground iron ore in the ratio of 1 part ore to 7 parts of graphitizer by weight. The ore contained 70%  $Fe_2O_3$ . This iron as cast had an ultimate tensile strength of 26,800 pounds per square inch, and its Brinell hardness number was 163. The depth of chill was reduced to 0.05 inch, and there was no evidence of pinhole porosity.

**Example 2.**—A medium hard iron containing 3.8% carbon and 2.1% silicon was made in a cupola under commercial foundry conditions and divided into three batches. The first batch was cast immediately. As cast its ultimate tensile strength was 27,400 pounds per square inch, and its Brinell hardness number was 179. The depth of chill was 0.22 inch. There was no evidence of pinhole porosity.

To the second batch was added 0.5% silicon just before casting by means of a ladle addition of the graphitizer used in Example 1. The iron was then cast. As cast its ultimate tensile strength was 20,300 pounds per square inch, its Brinell hardness number 156. The depth of chill was 0.06 inch, but there was considerable pinhole porosity.

The third batch was treated in the ladle just before casting with sufficient graphitizer to add 0.5% silicon, the same graphitizer being used but mixed with iron ore containing 70%  $Fe_2O_3$ , the ratio of ore to graphitizer being 1:7. The iron was then cast. Its ultimate tensile strength was 20,900 pounds per square inch, its Brinell hardness number 156. The depth of chill was 0.08 inch, and there was no evidence of pinhole porosity.

**Example 3.**—A hard iron containing 3.4% carbon and 1.8% silicon was made in a cupola under commercial conditions and divided into three batches. The first batch was cast immediately. It had a tensile strength of 35,600 pounds per square inch, its Brinell hardness number was 196, depth of chill was 0.94 inch, and there was no evidence of pinhole porosity.

To the second batch 0.5% silicon was added by means of a ladle addition of the graphitizer used in Example 1 just before casting. As cast the iron so treated had a tensile strength of 34,200 pounds per square inch and a Brinell hardness number of 187, and the depth of chill was 0.14 inch. There was considerable pinhole porosity.

The third batch was treated with graphitizer plus iron ore as the third batch in Example 2. The iron so treated had a tensile strength of 36,400 pounds per square inch and a Brinell hardness number of 196. The depth of chill was 0.13 inch, and there was no evidence of pinhole porosity.

In the following table the data obtained from the tests described in Examples 1, 2, and 3 are recapitulated for comparison. In the table "T. S." means ultimate tensile strength and is measured in pounds per square inch. "B. H. N." means Brinell hardness number.

Properties of cast irons made in Examples 1, 2, and 3

|             | T. S.  | B. H. N. | Chill Depth<br>Inches | Pinhole porosity |
|-------------|--------|----------|-----------------------|------------------|
| Example 1:  |        |          |                       |                  |
| Heat 1..... | 19,500 | 134      | 0.13                  | None.            |
| Heat 2..... | 24,300 | 146      | 0.06                  | Considerable.    |
| Heat 3..... | 26,800 | 163      | 0.05                  | None.            |
| Example 2:  |        |          |                       |                  |
| Heat 1..... | 27,400 | 179      | 0.22                  | Do.              |
| Heat 2..... | 20,300 | 156      | 0.06                  | Considerable.    |
| Heat 3..... | 20,900 | 156      | 0.08                  | None.            |
| Example 3:  |        |          |                       |                  |
| Heat 1..... | 35,600 | 196      | 0.94                  | Do.              |
| Heat 2..... | 34,200 | 187      | 0.14                  | Considerable.    |
| Heat 3..... | 36,400 | 196      | 0.13                  | None.            |

The results of these and other tests demonstrate that large additions of a graphitizer to molten cast iron effectively reduce the sensitivity of the iron when cast to variations in rate of cooling but that the iron may develop pinhole porosity. It is further shown that if the oxygen content of the molten iron is raised temporarily during the graphitizing treatment by mixing a metallic oxide with the graphitizer, the chill-reducing power of the graphitizer is not seriously detrimentally affected, and may even be improved, while the tendency of the iron to develop

pinhole porosity is substantially eliminated. The method of the invention accordingly makes possible heavy additions of graphitizers to molten cast iron without encountering the risk of developing pinhole porosity in the treated iron when cast.

If it is inconvenient or undesirable for any reason to add metallic oxides to the graphitizer used, the method of the invention may be practiced by oxidizing the graphitizer itself. For example, the graphitizer may be heated to a temperature of about 900° C. to 1000° C. in an oxidizing atmosphere for a time between about 10 or 15 minutes to 2 hours depending on the degree of oxidation desired.

In tests of this method of adding oxygen to molten iron samples of the same graphitizer used in Example 1 above were heated at 950° C. for 15 minutes, at 950° C. for 1 hour and at 1000° C. for 2 hours. The samples were calculated to have a total oxide content of 2.38%, 3.28%, and 4.16% respectively, after treatment. The oxidized graphitizers were then added, in an amount sufficient to add about 0.5% silicon, to a molten iron containing about 3.56% carbon and 1.91% silicon. No pinhole porosity was developed in the iron so treated, whereas the same iron to which had been added a similar amount of un-oxidized graphitizer had numerous pinholes. The depth of chill of the untreated iron was 0.56 inch; it was reduced to 0.13 inch in the iron treated with unoxidized graphitizer, to 0.14 inch in the iron treated with graphitizer containing 2.38% oxide, and to 0.17 inch in the iron treated with graphitizer containing 3.28% oxide. The depth of chill in the iron treated with graphitizer containing 4.16% oxide was 0.25 inch.

It will be apparent that the invention is not limited to the several specific examples cited herein by way of illustration of its principles. For example, it may be used with other graphitizers than those particularly mentioned, and other metallic oxides which are readily reducible in molten iron may be used to supply oxygen. The oxides used, although preferably in finely-divided form, may be used in briquetted form.

Modifications such as these of the method described herein are within the scope of the invention.

What is claimed is:

- 5 1. In the process of making cast iron which includes the step of adding to the molten cast iron a graphitizing agent comprising principally silicon and at least one strongly-deoxidizing graphitizing element, and containing a small amount of aluminum, whereby the cast iron is made desirably less sensitive to changes in chilling rate but undesirably susceptible to pinhole porosity, the method of counteracting such susceptibility to pinhole porosity without materially affecting such sensitivity to changes in chilling rate, which comprises adding to the molten cast iron, in admixture with the said graphitizing agent readily reducible metal-oxide material in an amount only sufficient to supply between one-half and five times the amount of oxygen theoretically required to combine with said aluminum.
- 10 2. Method as claimed in claim 1, wherein the metal-oxide material is iron oxide and wherein said iron oxide is added in an amount sufficient to supply about one-half to twice the amount of oxygen theoretically required to combine with all of said aluminum.
- 15 3. A method of treating molten cast iron which comprises adding to the molten iron a ferrosilicon containing at least about 0.25% aluminum and at least one strongly deoxidizing, graphitic-carbon promoting element, said ferrosilicon being added in a quantity sufficient to add about 0.1% to 1.5% silicon to the iron, and during the addition of said ferrosilicon temporarily raising the oxygen content of the molten iron by adding in admixture with said ferrosilicon at least one readily reducible metallic oxide in an amount only sufficient to supply about  $\frac{1}{2}$  to 5 times the amount of oxygen theoretically required to combine with all of the aluminum present in said ferrosilicon.

CHARLES O. BURGESS.  
HERMAN C. AUFDERHAAR.